

No. 669,698.

Patented Mar. 12, 1901.

E. IVINS.

PROCESS OF DRAWING METALLIC TUBES.

(Application filed June 4, 1900.)

(No Model.)

Fig. 1.



Fig. 2.



Fig. 3.



Fig. 4.



Witnesses

G. S. Elliott.  
M. Johnson

Inventor

Ellwood Ivins  
By Percy B. Hills  
Attorney

# UNITED STATES PATENT OFFICE.

ELLWOOD IVINS, OF PHILADELPHIA, PENNSYLVANIA, ASSIGNOR TO FRANK A. WILMOT, OF BRIDGEPORT, CONNECTICUT.

## PROCESS OF DRAWING METALLIC TUBES.

SPECIFICATION forming part of Letters Patent No. 669,698, dated March 12, 1901.

Application filed June 4, 1900. Serial No. 18,972. (No specimens.)

*To all whom it may concern:*

Be it known that I, ELLWOOD IVINS, a citizen of the United States, residing at Philadelphia, in the county of Philadelphia, State 5 of Pennsylvania, have invented new and useful Improvements in Processes of Drawing Metallic Tubes, of which the following is a specification.

My invention relates to the cold-drawing of 10 metallic tubes through dies, and has for its object to cheapen and expedite the operation of reducing or elongating the tube to the required finished dimensions, which object I accomplish by a process embracing a preliminary 15 annealing and pickling of the tube, a coating of the same designed to permit of any number of passes through the dies without any intermediate treatment whatsoever, the reduction of the tube by its passage 20 through dies and over mandrels, and finally the removal of the coating to restore the tube to its original condition.

In the accompanying drawings, Figure 1 is a sectional perspective view of a tube after 25 the preliminary annealing and pickling. Fig. 2 is a similar view of said tube coated. Fig. 3 is a similar view of said tube coated and after it has been drawn. Fig. 4 is a similar view of said tube drawn and with the coating 30 removed, the same being in a finished condition.

To the above end the treatment preliminary to drawing consists in first annealing the tube or hollow billet in the usual way, then dipping 35 the same in an acid solution to clear or remove the oxid or "scale" produced by the annealing, then dipping it in water to remove all traces of the acid solution, leaving it in the condition shown in Fig. 1, and finally 40 dipping it in a bath of molten soft metal, preferably a mixture of tin and lead in suitable proportions, to coat the tube both exteriorly and interiorly with said softer metal, as shown in Fig. 2. The tube so treated is 45 then drawn, preferably, over a fixed mandrel and through a fixed die to obtain the required reduction or elongation, and this drawing is repeated, but without intermediate annealings and without any intermediate fresh 50 coatings with the soft metal, over successively-smaller mandrels and through successively-smaller dies until the tube has attained the desired finished dimension, as shown in Fig.

3, it having been found that the coating of soft metal permits of this successive drawing 55 without intermediate annealings or intermediate fresh coatings with the soft metal, the same acting as a lubricant and not becoming hardened to the density of the die and mandrel, as would be the case with the surface of 60 the tube itself were it exposed to the action of the die and mandrel. After the drawing is finished the tube is then treated, either chemically or mechanically, to remove the soft-metal interior and exterior coating, thus 65 leaving said tube in its original condition, with no trace of the soft-metal coating employed in the process of drawing the same, as shown in Fig. 4. A further valuable result obtained is that any pittings that said tube may have 70 acquired during the preliminary annealing and pickling are thoroughly obliterated during the drawing, leaving the tube when the soft-metal coating is removed in a finished condition ready for use. 75

I am aware that it is not broadly new to coat a tube with soft metal to facilitate the passage thereof through a die, and such, therefore, I do not broadly claim; but I am not aware that tubes have been heretofore annealed and pickled, coated with soft metal, then drawn through successively-smaller dies and over successively-smaller mandrels without intermediate annealings or coatings, and finally treated to entirely remove said soft 85 metal, leaving the finished tube in its original condition. 80

Having thus described my invention, what I claim as new, and desire to secure by Letters Patent, is— 90

The herein-described process of drawing and finishing tubes, consisting in first annealing the same, then pickling the same, then coating the surfaces with antifriction metal, then drawing the same through suitable successively-smaller dies without any intermediate annealing or pickling or fresh coating 95 with soft metal, and finally removing the soft-metal coating, substantially as set forth.

In testimony whereof I have hereunto set 100 my hand in the presence of two subscribing witnesses.

ELLWOOD IVINS.

Witnesses:

LYNNE K. LEWIS,  
ELIZABETH FRICK.